

(No Model.)

A. L. & W. J. HUSTON.  
COMPOUND FOR COVERING BELT PULLEYS.

No. 520,992.

Patented June 5, 1894.



*d* {  
Ground Fibre  
Glue  
Rye Flour  
Alum  
Sal. Soda  
Borax  
Sal. Ammoniac  
Litharge  
Alcohol

WITNESSES.

Chas Ammon.

R. Schleicher.

INVENTORS.

A. L. & W. J. Huston  
By their Attorneys.

*Huston & Huston*

# UNITED STATES PATENT OFFICE.

ARTHUR L. HUSTON AND WILLIAM J. HUSTON, OF PHILADELPHIA,  
PENNSYLVANIA.

## COMPOUND FOR COVERING BELT-PULLEYS.

SPECIFICATION forming part of Letters Patent No. 520,992, dated June 5, 1894.

Application filed November 20, 1893. Serial No. 491,427. (No specimens.)

*To all whom it may concern:*

Be it known that we, ARTHUR L. HUSTON and WILLIAM J. HUSTON, both citizens of the United States, and residents of Philadelphia, Pennsylvania, have invented certain Improvements in Compounds for Covering Belt-Pulleys, of which the following is a specification.

The object of our invention is to provide a compound for application to the surface of driving pulleys for the purpose of strengthening the hold of the belt thereupon, and this object we attain in the manner hereinafter set forth, reference being had to the accompanying drawing which represents a transverse section of part of the rim of a pulley having the compound applied thereto.

Our compound, in the preferred form, is as follows: ground paper, rags, pulp, or like fibrous material, ten pounds; glue, two pounds; rye flour, one pound; sal soda, one ounce; sal ammoniac, one ounce; borax, one-half ounce; alum, one-half ounce; alcohol, one pint. These ingredients are mixed together in the form of a thick paste or mortar, sufficient water being added, if necessary, for the purpose. The face of the pulley is cleaned with lye or soap and water and then wiped dry and the compound is then spread upon the face of the pulley so as to form a layer of any desired thickness, this layer being shaped to give any desired amount of "crown" to the belt receiving surface of the pulley, and while the compound is still in a soft state fine wire is by preference wrapped around the pulley and drawn through the composition until it reaches the face of the pulley, the ends of the wire being properly secured and the layer of composition being then smoothed over to form a continuous surface, or wire gauze or like material may be used instead of the wrapped wire.

In the drawing *a* represents the rim of the pulley, *b* the wire wrapped around the same, and *c* the layer of composition forming the driving surface of the pulley.

The ground paper or other fibrous material constitutes the bulk or body of our improved composition, the glue, rye flour and alum being used as a cement for the purpose of uniting the fibrous particles in a coherent and homogeneous mass. The sal-soda and borax

being salts having a tendency to absorb moisture, serve to temper the compound and prevent it from becoming brittle or friable when it is used in places where the air is very dry. 55 The function of the sal-ammoniac is to cause the rusting or oxidizing of the face of the pulley and its wire wrapping so as to increase the hold of the composition upon the same. The litharge has the effect of hardening the 60 composition, and the alcohol is employed for the purpose of hastening the drying of the layer of compound after the same has been applied to the face of the pulley and also for the purpose of preventing the compound 65 from becoming sour when exposed to the air.

When the compound is intended for use in places where the air is always more or less charged with moisture, the use in the compound of the absorbent salts, such as sal-soda 70 or borax may not be necessary, and while we prefer the use of the glue, rye flour and alum as the cementing medium for uniting the fibrous particles of the compound, other cementing or uniting agents soluble in water might be employed without departing from the main features of our invention, and other oxidizing agents than sal-ammoniac may be availed of, while in cases where the properties imparted to the compound by the litharge and alcohol 75 80 are not important, these ingredients may be omitted. The proportions of the ingredients may also be varied within considerable limits, depending upon the desired possession by the compound in greater or less measure of 85 the qualities which the various ingredients serve to impart to said compound.

Having thus described our invention, we claim and desire to secure by Letters Patent—

1. The within described compound for forming the driving surface of a pulley, said compound consisting of a cohering homogeneous mortar-like mass of ground fibrous material and a cementing agent soluble in water, substantially as specified. 90

2. The within described compound for forming the driving surface of a pulley, said compound consisting of ground fibrous material, a cementing agent soluble in water, and an absorbent of moisture, such as sal-soda or borax, substantially as specified. 95 100

3. The within described compound for form-

ing the driving surface of a pulley said compound consisting of fibrous material, a cementing agent soluble in water, and an oxidizing agent, such as sal-ammoniac, the whole 5 constituting a coliering, homogeneous, mortar-like mass substantially as specified.

4. The within described compound for forming the driving surface of a pulley, said compound consisting of fibrous material, a cementing agent, and litharge, substantially as 10 specified.

5. The within described compound for forming the driving surface of a pulley, said com-

pound consisting of fibrous material, a cementing agent, a moisture absorbent, such as 15 sal-soda or borax, an oxidizing agent, such as sal-ammoniac, and a hardening material, such as litharge, substantially as specified.

In testimony whereof we have signed our names to this specification in the presence of 20 two subscribing witnesses.

ARTHUR L. HUSTON.  
WILLIAM J. HUSTON.

Witnesses:

FRANK BECHTOLD,  
JOSEPH H. KLEIN.